

Sept. 2, 1947.

D. MAPES

2,426,630

HIGH PRESSURE GASEOUS OXYGEN PACKAGE

Filed Sept. 27, 1943



INVENTOR.

*Daniel Mapes*

BY

*Ernest A. Jensen*

ATTORNEY

Patented Sept. 2, 1947

2,426,630

# UNITED STATES PATENT OFFICE

2,426,630

## HIGH-PRESSURE GASEOUS OXYGEN PACKAGE

Daniel Mapes, West Caldwell, N. J., assignor to Specialties Development Corporation, Bloomfield, N. J., a corporation of New Jersey

Application September 27, 1943, Serial No. 504,065

1 Claim. (Cl. 206—0.6)

1

The present invention relates to metallic containers, and more particularly to containers for storing fluid media under pressure.

Heretofore, it has been customary to store various kinds of fluid medium in ordinary alloy or carbon type steel containers or the like at pressure of between about 700 and about 2200 pounds per square inch. These containers are used extensively in connection with vehicles and craft for carrying on warfare, and are likely to be subjected to gunfire when in combat areas. In many cases the containers are utilized for storing a fluid medium capable of supporting combustion. When such containers are pierced by a projectile from a machine gun or the like, the impact of the projectile heats the metal sufficiently to cause it to burn in the presence of the combustion supporting medium. The burning of the metal may cause splashing of molten metal or a burst of flame which sets afire the vehicle or craft wherein the containers are used.

An object of the present invention is to provide metallic containers for storing fluid media capable of supporting combustion at relatively high pressures, the wall surface of the containers being covered with a metal adapted to minimize burning of the containers in the event the containers are pierced by a projectile from a machine gun or the like.

Another object is to provide a portable container for high pressure fluid media adapted to support combustion, which can be fired upon without the occurrence of severe flashing or burning.

A further object is to greatly minimize and to eliminate the fire hazard in vehicles and craft carrying containers storing high pressure media which are capable of supporting combustion.

Other and further objects of the invention will be obvious upon an understanding of the illustrative embodiment about to be described, or will be indicated in the appended claims, and various advantages not referred to herein will occur to one skilled in the art upon employment of the invention in practice.

In accordance with the invention, it has been found that the foregoing objects can be accomplished by forming the containers of a metal which will burn rapidly when subjected to heat in the presence of oxygen, the wall surface of the containers being covered with a metal, which, when in intimate contact with compressed oxygen and subjected to high temperature due to the container walls being pierced by gunfire or the like, will fuse and oxidize rapidly to form a protective metallic oxide coating serving to prevent burning of the containers beyond the point at which the walls are pierced. Such metals may be copper and copper alloys.

Suitable copper alloys are those of the copper-

2

nickel type, containing 60 to 70% nickel and 25 to 35% copper; the copper-beryllium type, containing 96 to 98% copper and 2 to 4% beryllium; and the copper-nickel-beryllium type, containing 25 to 5% nickel, 2 to 2.75% beryllium and the balance copper. At high temperatures copper and copper alloys are rapidly coated with corresponding oxides thereof which are difficult to burn.

10 In the accompanying drawing the single figure is an elevational view, partly in section, illustrating a container in accordance with the present invention.

In the drawing there is shown a container 10 having a neck 11 formed with an opening for receiving a valve 12 or the like. The container has a wall 14 provided with interior and exterior surface layers or coatings 15 and 16, respectively, as about to be described.

15 It has been found that burning of the containers could be prevented by constructing them of any suitable metal, including ordinary alloy or carbon type steels, aluminum or aluminum alloys, and providing the interior and exterior walls with a surface layer or coating of copper or such copper alloys. This protective layer may be applied to the surface of the metal from which the containers are to be formed, or may be applied to the containers after they have been formed by any suitable methods such as spraying molten metal thereon, or positioning a sheet of protective metal adjacent thereto.

20 The containers formed of the foregoing described materials may be of any desired size and 35 may be of any conventional shape, such as generally cylindrical or spherical. The containers preferably are designed to safely store the fluid medium at working pressures of between about 700 to about 2200 pounds per square inch or even more, and to resist shattering when struck by gunfire or the like.

25 The fluid medium stored in the containers usually is oxygen adapted to be used on aircraft for breathing purposes during high altitude flights. Normally, when a projectile pierces the walls of a container in which oxygen is stored, the impact of the projectile generates heat. This causes heating of the wall of the container adjacent the entrance and exit holes of the projectile to a temperature sufficiently high to ignite the metal. The oxygen rushing out of the holes formed in the container tends to support the combustion of the metal for a substantial period. When the containers are covered with the protective materials described herein, such burning is negligible or is eliminated, as will be pointed out in greater detail in the examples about to follow.

30 In addition to safely storing oxygen, the containers in accordance with the present invention are adapted to be utilized for storing other fluid

media capable of supporting combustion, for example, compressed air.

The following examples illustrate the invention:

*Example I.*

A cylindrical shell formed of ordinary low alloy type steel generally used for making cylinders was internally coated with a spray of molten copper by employing a process developed by Metallizing Engineering Company of Long Island City, New York, known as "metallizing." The shell was then formed into a cylindrical container which was sprayed externally with copper by employing the "metallizing" process. An internal and external surface layer of copper having a thickness of about .01 of an inch was applied to the container by this process.

The cylindrical wall of the container was provided with a winding of two layers of music wire, as shown in my prior Patent No. 2,370,677. The container had a capacity of about 295 cubic inches, and was filled with oxygen at 1800 pounds per square inch pressure.

The container was fired at by a .50 caliber machine gun using 2700 feet per second velocity, armor piercing ammunition, at a range of 75 yards.

When the projectile struck the container the amount of flashing and burning was greatly minimized as compared with uncoated containers of the same material as the container tested. The copper was oxidized at the entrance and exit holes which retarded burning of the steel.

With surface layers or coatings of copper nickel alloys and copper-beryllium alloys resistance to burning also is increased. Flashing and burning can be further minimized by increasing the thickness of the coating.

*Example II*

A cylindrical shell similar to the shell utilized in connection with the test described in Example I was provided with a lining at the interior thereof. The lining was in the form of a cylindrical tube formed of copper sheeting  $\frac{1}{16}$  of an inch thick. The tube was forced into the shell so that it contacted the inner cylindrical wall of the shell and formed a protective covering therefor. The shell was then formed into a cylindrical container which was wire-wound like the container mentioned in Example I.

The container provided had a capacity of about 295 cubic inches, and was filled with oxygen at 1800 pounds per square inch pressure.

The container was fired at by a .50 caliber machine gun using 2700 feet per second velocity, armor piercing ammunition, at a range of 75 yards.

When the projectile struck the container, it pierced the outer wall fired upon and exited through the opposite wall. The amount of flashing and burning was very slight and was considerably less than in connection with the container described in Example I, thus demonstrating that layers of copper sheeting as well as surface coatings greatly minimize flashing and burning.

Sheeting of copper alloys containing nickel and/or beryllium has good resistance to burning and can be utilized to obtain similar results.

From the foregoing description and examples, it will be seen that the present invention provides improved high pressure containers for

storing fluid media capable of supporting combustion. By rendering the containers resistive to burning in the presence of a combustion supporting medium, the fire hazards in vehicles and craft on which the containers are used are greatly minimized, thus increasing the safety of its occupants. The containers in accordance with the invention can be readily manufactured at but a slight increase in cost to attain the foregoing advantages which fully justify such increase in cost.

It will be understood that the details and examples hereinbefore set forth are illustrative only, and that the invention as broadly described and claimed, is in no way limited thereby.

It is also to be understood that the following claim is intended to cover all the generic and specific features of the invention herein described, and all statements of the scope of the invention which, as a matter of language, might be said to fall therebetween.

I claim:

A portable sealed package comprising a metallic container containing a supply of gaseous oxygen compressed to at least 700 pounds per square inch which supply is adapted to be dispensed from the container, said container being formed of a metal which will burn rapidly when subjected to heat in the presence of oxygen and having the interior and exterior wall surface thereof covered with a fusible and rapidly oxidizable material selected from the group consisting of copper, copper-nickel alloys and copper-beryllium alloys, which materials, when in intimate contact with the compressed oxygen and subjected to high temperature due to the container wall being pierced by gunfire or the like, will fuse and oxidize rapidly to form a protective metallic oxide coating serving to prevent burning of the container beyond the point at which the container is pierced.

DANIEL MAPES.

REFERENCES CITED

The following references are of record in the file of this patent:

UNITED STATES PATENTS

| Number    | Name              | Date           |
|-----------|-------------------|----------------|
| 2,205,708 | Zurbrugg          | June 25, 1940  |
| 1,544,854 | Mueller et al.    | July 7, 1925   |
| 2,329,765 | Jackson et al.    | Sept. 21, 1943 |
| 2,337,049 | Jackson           | Dec. 21, 1943  |
| 2,127,712 | Bart              | Aug. 23, 1938  |
| 2,042,426 | Kinzel            | May 26, 1936   |
| 2,339,554 | Kuhn              | Jan. 18, 1944  |
| 2,344,856 | Earle             | Mar. 21, 1944  |
| 1,961,117 | Wall              | May 29, 1934   |
| 1,995,616 | Kamack            | Mar. 26, 1935  |
| 2,245,430 | Courtright et al. | June 10, 1941  |
| 280,905   | Brownell          | July 10, 1883  |

FOREIGN PATENTS

| Number  | Country       | Date          |
|---------|---------------|---------------|
| 376,822 | Great Britain | July 18, 1932 |

OTHER REFERENCES

Metals Handbook, 1936 edition, published by American Society for Metals, 7016 Euclid Ave., Cleveland, Ohio.

Alloys of Chromium and Nickel, by Kinzel and Franks, first edition, published by McGraw-Hill Book Co., New York.